

April 20, 1971

YOSHINOBU MURAKAMI ET AL

3,575,698

ELECTROPHOTOGRAPHIC MATERIAL

Filed June 17, 1968

3 Sheets-Sheet 1



Fig. 1 .Brominated poly-N-vinylcarbazole



Fig. 2 .Brominated poly-N-vinylcarbazole+compound 2



Fig. 3 .Brominated poly-N-vinylcarbazole+compound 13



Fig. 4 .Brominated poly-N-vinylcarbazole+compound 23

YOSHINOBU MURAKAMI AND  
KAZUHISA MORIMOTO, INVENTORS

By: Wendroth, Lind & Ponack, Attorneys

April 20, 1971

YOSHINOBU MURAKAMI ET AL

3,575,698

ELECTROPHOTOGRAPHIC MATERIAL

Filed June 17, 1968

3 Sheets-Sheet 2



Fig. 5 Poly-N-vinylcarbazole



Fig. 6 Poly-N-vinylcarbazole+compound 3



Fig. 7 Poly-N-vinylcarbazole+compound 11



Fig. 8 Poly-3,6-dibromo-N-vinylcarbazole

YOSHINOBU MURAKAMI AND  
KAZUHISA MORIMOTO, INVENTORS

By: Wenderoth, Lind & Ponack,  
Attorneys

April 20, 1971

YOSHINOBU MURAKAMI ET AL

3,575,698

ELECTROPHOTOGRAPHIC MATERIAL

Filed June 17, 1968

3 Sheets-Sheet 3



Fig. 9 Poly-3,6-dibromo-N-vinylcarbazole+compound 14



Fig. 10 Poly-3,6-dibromo-N-vinylcarbazole+compound 16



Fig. 11 Brominated poly-N-vinylcarbazole+compound 11,  
13, 14

YOSHINOBU MURAKAMI AND  
KAZUHISA MORIMOTO, INVENTORS

By: Wenderoth, Lind & Ponack, Attorneys

3,575,698

## ELECTROPHOTOGRAPHIC MATERIAL

Yoshinobu Murakami and Kazuhisa Morimoto, Osaka, Japan, assignors to Matsushita Electric Industrial Co., Ltd., Osaka, Japan

Filed June 17, 1968, Ser. No. 737,787

Claims priority, application Japan, Aug. 1, 1967,  
42/49,661

Int. Cl. G03g 5/06

U.S. Cl. 96—1.6

5 Claims

### ABSTRACT OF THE DISCLOSURE

An improved electrophotographic material comprising a conductive support layer and a photoconductive insulating layer, the latter comprising a combination of a photoconductive poly-compound and a carbonium salt as novel sensitizer, said photoconductive polymeric compound comprising at least one of poly-N-vinylcarbazole, poly-3,6-dibromo-N-vinylcarbazole, brominated poly-N-vinylcarbazole, polyacenaphthylene and polyvinylanthracene.

This invention relates to novel light-sensitive layers and more particularly to electrophotographic light-sensitive polymer layers containing a carbonium salt as a novel sensitizer of organic photoconductors.

Various light-sensitive layers are well known in the electrophotographic art for making copies of documents, drawings, transparencies, etc. These layers contain an organic photoconductive compound, such as poly-N-vinylcarbazole, poly-3,6-dibromo-N-vinylcarbazole, brominated poly-N-vinylcarbazole, polyacenaphthylene, polyvinylanthracene, etc. These layers are non-conductors of electricity before exposure and become electrical conductors upon exposure.

It is necessary for the electrophotographic art that the photoconductive material has a high photoconductivity in the long wavelength region of the visible spectrum. Such a photoconductive material makes it possible for the electrophotographic art to employ inexpensive and convenient light sources such as incandescent lamps in a reduced exposure time and to reproduce colored pictures. The photoconductive materials mentioned above, however, have usually a low photoconductivity and spectrum characteristics sensitive to the short wavelength region of the exposure light and do not satisfy entirely the above requirement.

It is known that an addition of a so-called sensitizer can improve photoconductivity and spectrum characteristics of the above photoconductive compounds. Conventional sensitizers are dyestuff compounds, such as triarylmethane dyes, xanthene dyes, triazine dyes or acridine dyes, but the conventional sensitizers are not entirely satisfactory for improving the photoconductivity and the spectrum characteristics of the available photoconductive compounds.

In addition to the high photoconductivity and spectrum characteristics sensitive to visible light, the electrophotographic art requires a high electric resistance of photoconductive materials in the dark. Conventional sensitizers are apt to increase the dark conductivity whereas they promote the photoconductivity. A high dark conductivity of photoconductive materials is not desirable because it results in a loss of the applied electrostatic charge in the dark.

An object of the invention is to provide electrophotographic materials having a high photoconductivity and spectrum characteristics sensitive to a long wavelength region of the visible spectrum.

Another object of the invention is to provide electro-

photographic materials having a high electric resistance in the dark.

These and other objects are accomplished by adding a carbonium salt as a sensitizer to poly-N-vinylcarbazole, poly-3,6-dibromo-N-vinylcarbazole, brominated poly-N-vinylcarbazole, polyacenaphthylene or polyvinylanthracene, as a light-sensitizing film-forming composition.

The invention is further explained in the following description with reference to the accompanying drawings 10 wherein:

FIG. 1 represents the wedge spectrogram for an electrophotographic material coated with an unsensitized solution of 10 weight percent of brominated poly-N-vinylcarbazole in chlorobenzene.

FIG. 2 represents the wedge spectrogram for an electrophotographic material coated with a solution containing 10 weight percent of brominated poly-N-vinylcarbazole, and, as a sensitizer, 0.04 weight percent of tris(4-methoxyphenyl)carbonium perchlorate, said brominated poly-N-vinylcarbazole being dissolved in a solvent of four weight parts of chlorobenzene and one weight part of dichloroethane.

FIG. 3 represents the wedge spectrogram for an electrophotographic material coated with a solution containing 10 weight percent of brominated poly-N-vinylcarbazole, and, as a sensitizer, 0.04 weight percent of bis(4-methoxyphenyl)-2'-methoxynaphthyl(1')carbonium perchlorate, said brominated poly-N-vinylcarbazole being dissolved in a solvent of four weight parts of chlorobenzene and one weight part of dichloroethane.

FIG. 4 represents the wedge spectrogram for an electrophotographic material coated with a solution containing 10 weight percent of brominated poly-N-vinylcarbazole, and, as a sensitizer, 0.04 weight percent of bis(4-methoxyphenyl)- $\omega$ -phenylbutadienylcarbonium perchlorate, said brominated poly-N-vinylcarbazole being dissolved in a solvent of four weight parts of chlorobenzene and one weight part of dichloroethane.

FIG. 5 represents the wedge spectrogram for an electrophotographic material coated with an unsensitized solution of 10 weight percent of poly-N-vinylcarbazole in chlorobenzene.

FIG. 6 represents the wedge spectrogram for an electrophotographic material coated with a solution containing 10 weight percent of poly-N-vinylcarbazole, and, as a sensitizer, 0.04 weight percent of bis(4-methoxyphenyl)naphthyl(1')carbonium perchlorate, said poly-N-vinylcarbazole being dissolved in a solvent of four weight parts of chlorobenzene and one weight part of dichloroethane.

FIG. 7 represents the wedge spectrogram for an electrophotographic material coated with a solution containing 10 weight percent of poly-N-vinylcarbazole, and, as a sensitizer, 0.04 weight percent of phenyl(4-methoxyphenyl)-4'-methoxynaphthyl(1')carbonium perchlorate, said poly-N-vinylcarbazole being dissolved in a solvent of four weight parts of chlorobenzene and one weight part of dichloroethane.

FIG. 8 represents the wedge spectrogram for an electrophotographic material coated with an unsensitized solution of 10 weight percent of poly-3,6-dibromo-N-vinylcarbazole in chlorobenzene.

FIG. 9 represents the wedge spectrogram for an electrophotographic material coated with a solution containing 10 weight percent of poly-3,6-dibromo-N-vinylcarbazole, and, as a sensitizer, 0.04 weight percent of phenyl(4-methoxyphenyl)2'-methoxynaphthyl(1')carbonium perchlorate, said poly-3,6-dibromo-N-vinylcarbazole being dissolved in a solvent of four weight parts of chlorobenzene and one weight part of dichloroethane.

FIG. 10 represents the wedge spectrogram for an electrophotographic material coated with a solution contain-

ing 10 weight percent of poly-3,6-dibromo-N-vinylcarbazole, and, as a sensitizer, 0.04 weight percent of bis(4-methoxyphenyl)phenanthryl(9')carbonium perchlorate, said poly-3,6-dibromo-N-vinylcarbazole being dissolved in a solvent of four weight parts of chlorobenzene and one weight part of dichloroethane.

FIG. 11 represents the wedge spectrogram for an electrophotographic material coated with a solution containing 10 weight percent of brominated poly-N-vinylcarbazole, and, as sensitizers, 0.024 weight percent of phenyl(4-methoxyphenyl)-4'-methoxynaphthyl(1')carbonium perchlorate, 0.012 weight percent of bis(4-methoxyphenyl)-2'-methoxynaphthyl(1')carbonium perchlorate and 0.024 weight percent of phenyl(4-methoxyphenyl)-2'-methoxynaphthyl(1')carbonium perchlorate, said brominated poly-N-vinylcarbazole being dissolved in a solvent of four weight parts of chlorobenzene and one weight part of dichloroethane.

The carbonium salt compound (sensitizer) according to the present invention has the following formula:



wherein

$R_1$ ,  $R_2$ ,  $R_3$  each is an aliphatic group such as styryl, 2-methoxystyryl, 4-methoxystyryl or  $\omega$ -phenylbutadienyl, phenyl or 4-biphenyl, alkoxyphenyl such as 2-methoxyphenyl, 4-methoxyphenyl, 4-ethoxyphenyl, 3,4-dimethoxyphenyl or 3,4-diethoxyphenyl, phenoxyphenyl, naphthyl, alkoxyphenyl such as 2-methoxynaphthyl, 4-methoxynaphthyl, 2-ethoxynaphthyl or 4-ethoxynaphthyl, anthryl, alkoxyanthryl, phenanthryl or alkoxyphenanthryl.

Anion is anionic function selected from the group consisting of fluoborate, chloride, iodide, perchlorate, chloroferrate and chlorozincate.

The carbonium salts are prepared generally by one of two methods. A first method is based on the reaction of a Grignard reagent (I) in ether or in a mixed solvent of ether and benzene with a ketone compound (II). After the reaction product is hydrolyzed with an aqueous solution of ammonium chloride, the product (III) is treated with perchloric acid to obtain perchlorate (IV) in the presence of acetic acid and acetic anhydride. This reaction is shown by the following chemical equation:



A second method is achieved by the reaction of carbinol intermediate (V) containing a methylene group, with an aromatic aldehyde (VI) in the presence of perchloric acid and hydrogen chloride. This reaction product (VII) is characterized by an ethenyl linkage. This reaction is shown by the following chemical equation:



Representative examples of the carbonium salts according to the invention are listed in Table 1.

4  
TABLE 1

| Compound Number | Name of compound                                                                                     |
|-----------------|------------------------------------------------------------------------------------------------------|
| 1               | Bis(4-methoxyphenyl)styrylcarbonium perchlorate.                                                     |
| 2               | Tris(4-methoxyphenyl)carbonium perchlorate.                                                          |
| 3               | Bis(4-methoxyphenyl)naphthyl(1')carbonium perchlorate.                                               |
| 4               | Tris(4-methoxyphenyl)carbonium chloroferrate.                                                        |
| 5               | Diphenyl-naphthyl(1')carbonium perchlorate.                                                          |
| 6               | Phenyl(4-ethoxynaphthyl(1'))carbonium perchlorate.                                                   |
| 7               | Phenyl(4-methoxynaphthyl(1'))naphthyl(1')carbonium perchlorate.                                      |
| 8               | Phenyl-biphenyl(4)naphthyl(1')carbonium perchlorate.                                                 |
| 9               | Phenyl-bis(4-methoxyphenyl)carbonium chloroferrate.                                                  |
| 10              | Phenyl(3,4-dimethoxyphenyl)biphenyl(4')carbonium perchlorate.                                        |
| 11              | Phenyl(4-methoxyphenyl)-4'-methoxynaphthyl(1')carbonium perchlorate.                                 |
| 12              | Phenyl-bis(4-ethoxynaphthyl)carbonium perchlorate.                                                   |
| 13              | Bis(4-methoxyphenyl)-2'-methoxynaphthyl(1')carbonium perchlorate.                                    |
| 14              | Phenyl(4-methoxyphenyl)-2'-methoxynaphthyl(1')carbonium perchlorate.                                 |
| 15              | Phenyl-biphenyl(4)-2'-methoxynaphthyl(1')carbonium perchlorate.                                      |
| 16              | Bis(4-methoxyphenyl)phenanthryl(9')carbonium perchlorate.                                            |
| 17              | Phenyl(3,4-diethoxynaphthyl)phenanthryl(9')carbonium perchlorate.                                    |
| 18              | Phenyl(4-methoxynaphthyl(1))phenanthryl(9')carbonium chloroferrate.                                  |
| 19              | Bis(4-methoxyphenyl)-4'-phenoxyphenylcarbonium fluoborate.                                           |
| 20              | Phenyl(4-ethoxyphenyl)-4'-phenoxyphenylcarbonium perchlorate.                                        |
| 21              | Phenyl(4-phenoxyphenyl)-4'-methoxynaphthyl(1')carbonium perchlorate.                                 |
| 22              | Bis(4-methoxyphenyl)-4'-methoxystyrylcarbonium perchlorate.                                          |
| 23              | Bis(4-methoxyphenyl)- $\omega$ -phenylbutadienylcarbonium perchlorate.                               |
| 24              | Bis(4-methoxyphenyl)- $\alpha$ -(4'-methoxyphenyl)-4''-methoxystyrylcarbonium perchlorate.           |
| 25              | Bis(4-methoxyphenyl)- $\alpha$ -(4'-methoxyphenyl)- $\omega$ -phenylbutadienylcarbonium perchlorate. |
| 26              | Phenyl-bis(4-methoxyphenyl)carbonium perchlorate.                                                    |
| 27              | Diphenyl(4-methoxyphenyl)carbonium perchlorate.                                                      |
| 28              | Triphenylcarbonium perchlorate.                                                                      |
| 29              | Phenyl(4-methoxyphenyl)naphthyl(1')carbonium perchlorate.                                            |
| 30              | Phenyl(4-methoxyphenyl)biphenyl(4')carbonium perchlorate.                                            |
| 31              | Phenyl(4-methoxyphenyl)phenanthryl(9')carbonium perchlorate.                                         |
| 32              | Phenyl(4-methoxynaphthyl(1))phenanthryl(9')carbonium perchlorate.                                    |
| 33              | Phenyl-biphenyl(4)phenanthryl(9')carbonium perchlorate.                                              |
| 34              | Bis(4-methoxyphenyl)-4'-phenoxyphenylcarbonium perchlorate.                                          |
| 35              | Phenyl(4-methoxyphenyl)-4'-phenoxyphenylcarbonium perchlorate.                                       |
| 36              | Phenyl-biphenyl(4)-4'-phenoxyphenylcarbonium perchlorate.                                            |
| 37              | Tris(4-methoxyphenyl)carbonium iodide.                                                               |
| 38              | Tris(4-methoxyphenyl)carbonium chlorozincate.                                                        |
| 39              | Tris(4-methoxyphenyl)carbonium fluoroborate.                                                         |
| 40              | Tris(4-methoxyphenyl)carbonium chloride.                                                             |

Table 2 lists additional information on the color in dichloroethane and melting point of the novel compounds according to the invention.

TABLE 2

| Compound Number | Color in dichloroethane | Melting point (°C.) |
|-----------------|-------------------------|---------------------|
| 1               | Reddish violet          | 93-95               |
| 2               | Reddish orange          | 102-103             |
| 3               | Reddish violet          | 1162                |
| 4               | Reddish orange          | 168-169             |
| 5               | Brown                   | 1287                |
| 7               | Reddish orange          | 1241                |
| 8               | Violet                  | >300                |
| 9               | Reddish orange          | 131-132             |
| 11              | Greenish blue           | 1135                |
| 13              | Reddish violet          | 1162                |
| 14              | Greenish yellow         | 1141                |
| 15              | Red                     | >300                |
| 16              | Reddish violet          | 139-143             |
| 21              | Greenish blue           | 121-123             |
| 22              | Reddish violet          | 135-137             |
| 23              | Violet                  | 158-161             |
| 24              | Reddish orange          | >300                |
| 25              | Red                     | 1282                |
| 26              | Orange                  | 210-212             |
| 27              | do                      | 194-195             |
| 28              | Yellow                  | 154-157             |
| 29              | Reddish orange          | 123-126             |
| 30              | Red                     | 132-134             |
| 31              | Red                     | 127-130             |
| 32              | Reddish orange          | 247-249             |
| 33              | Reddish violet          | 1262                |
| 34              | Reddish orange          | 108-112             |
| 35              | do                      | 85-88               |
| 36              | Red                     | 98-102              |
| 37              | Reddish orange          | 148-149             |
| 38              | do                      | 234-235             |
| 39              | do                      | 188-190             |
| 40              | do                      | 147-148             |

75 <sup>1</sup> Decompose.

A simple per se well known exchange reaction makes it possible for the anionic function of the carbonium salt compounds to consist of  $\text{Cl}^-$ ,  $\text{I}^-$ ,  $\text{BF}_4^-$ ,  $\text{ZnCl}_3^-$ ,  $\text{FeCl}_4^-$  or  $\text{ClO}_4^-$ .

The following description will explain a practical method for making carbonium salts with reference to exemplary compounds. The details of the preparation of other compounds will be apparent to the skilled in the art from the preceding disclosure and the following illustrative examples of preparation methods of various compounds according to the invention:

(a) Bis(4-methoxyphenyl)styrylcation perchlorate (compound No. 1)



To a Grignard reagent prepared from 18 grams of  $\beta$ -bromostyrene, 2.4 grams of magnesium and a small amount of iodine in 50 milliliters of dry ether, there are slowly added 5 grams of  $p,p'$ -dimethoxybenzophenone. The solution is then refluxed for 2 hours and poured into an aqueous solution of ammonium chloride to hydrolyze the reaction product. The ether solution of the product is dried with anhydrous sodium sulfate. The solution is filtered and diluted with ether to 300 milliliters. To the solution, there are added 10 milliliters of acetic acid and 10 milliliters of acetic anhydride, then the solution is cooled and treated slowly with 6 milliliters of 60% perchloric acid. Precipitated crystals are filtered off, washed with ether and dried to obtain 4.3 grams of red crystals having a melting point of 93° to 95° C.

(b) Tris(4-methoxyphenyl)carbonium perchlorate (compound No. 2) and chloroferrate (compound No. 4)



To a Grignard reagent prepared from 2.8 grams of  $\beta$ -bromoanisole, 0.36 gram of magnesium and a small amount of iodine in 10 milliliters of dry ether, there are slowly added 2.5 grams of  $p,p'$ -dimethoxybenzophenone. The solution is then refluxed for 1 hour and poured into an aqueous solution of ammonium chloride to hydrolyze the reaction product. The ether solution of the product is dried with anhydrous sodium sulfate. The solution is filtered and diluted with ether to 300 milliliters. To the solution, there are added 10 milliliters of acetic acid and 10 milliliters of acetic anhydride, and then the solution is cooled and treated slowly with 3 milliliters of 60% perchloric acid. Precipitated crystals are collected, washed with ether and recrystallized twice from acetic acid to obtain 2.3 grams of reddish orange crystals of perchlorate which have a melting point of 192° to 193° C.

Furthermore, 1 gram of the crystals is dissolved in 30 milliliters of concentrated hydrochloric acid, and suc-

cessively, 20 milliliters of acetic acid. To the solution are added 30 milliliters of concentrated hydrochloric acid containing 5 grams of ferric chloride, then precipitated crystals are collected and recrystallized from acetic acid to obtain 0.9 gram of chloroferrate crystals having a melting point of 168° C. to 169° C.

(c) Phenyl - bis(4 - methoxyphenyl)carbonium perchlorate (compound No. 26) and chloroferrate (compound No. 9)

10



To a Grignard reagent prepared from 4.7 grams of  $p$ -bromoanisole, 0.6 gram of magnesium and a small amount of iodine in 15 milliliters of dry ether, there are slowly added 3.4 grams of  $p$ -methoxybenzophenone. After the solution is then refluxed for 1 hour, the solution is hydrolyzed by being poured into an aqueous solution of ammonium chloride. The ether solution is dried with anhydrous sodium sulfate, after which 100 milliliters of ether are added to the solution, followed by 10 milliliters of acetic acid and 10 milliliters of acetic anhydride; then the solution is cooled and treated slowly with 3 milliliters of 60% perchloric acid. Precipitated crystals are collected, washed with ether and recrystallized from a mixed solvent of acetic acid and dichloroethane (5:1). The crystals of perchlorate thus obtained have a melting point of 210° to 212° C.

Furthermore, 0.5 gram of the crystals is dissolved in 15 milliliters of concentrated hydrochloric acid and, successively, 15 milliliters of acetic acid. To the solution, then are added 2.5 grams of ferric chloride dissolved in 15 milliliters of concentrated hydrochloric acid. The precipitated crystals are collected and recrystallized from acetic acid. The amount of the crystals is 0.4 gram. The needle-like crystals of chloroferrate obtained have a melting point of 131° to 132° C.

(d) Bis(4-methoxyphenyl)-2'-methoxynaphthyl(1') carbonium perchlorate (compound No. 13)



To a Grignard reagent prepared from 6 grams of  $\alpha$ -bromo- $\beta$ -methoxynaphthalene, 0.6 gram of magnesium and a small amount of iodine in 20 milliliters of dry ether and 10 milliliters of dry benzene, there are slowly added 3.8 grams of  $p,p'$ -dimethoxybenzophenone. After the solution is then refluxed for 1 hour, the solution is poured into an aqueous solution of ammonium chloride. The ether solution is dried with anhydrous sodium sulfate and then 100 milliliters of ether are added to the solution followed by 10 milliliters of acetic acid and, successively, 10 milliliters of acetic anhydride; then the solution is treated slowly with 3 milliliters of 60% perchloric acid. Precipitated crystals are collected and reprecipitated again by pouring the dichloro ethane solution into ether. The crystals of perchlorate thus obtained have a decom-

posing point of 162° C. The amount of the crystals is 3.7 grams.

(e) Phenyl(4-phenoxyphenyl)-4'-methoxynaphthyl (1')carbonium perchlorate (compound No. 21)



To a Grignard reagent prepared from 6.2 grams of p-bromo-diphenylether, 0.6 gram of magnesium and a small amount of iodine in 20 milliliters of dry ether, there are slowly added 4.2 grams of 1-benzoyl-4-methoxynaphthalene in 20 milliliters of dry ether. After the solution is then refluxed for 1 hour, the solution is hydrolyzed by being poured into an aqueous solution of ammonium chloride. The ether solution is dried with anhydrous sodium sulfate, after which 100 milliliters of ether are added to the solution. To the latter, there are then added 10 milliliters of acetic acid and 10 milliliters of acetic anhydride, and then the solution is treated slowly with 3 milliliters of 60% perchloric acid. Precipitated crystals are collected and reprecipitated from the dichloroethane solution by means of ether. The crystals of perchlorate thus obtained have a melting point of 121° to 123° C. The amount of the crystals is 1.5 grams.

(f) Bis(4-methoxyphenyl)- $\omega$ -phenylbutadienylcarbonium perchlorate (compound No. 23)



To a Grignard reagent prepared from 9.4 grams of p-bromoanisole, 1.2 grams of magnesium and a small amount of iodine in 30 milliliters of dry ether, there are slowly added 4.8 grams of p-methoxyacetophenone in 20 milliliters of dry ether. After the solution is then refluxed for 1 hour, the solution is poured into an aqueous solution of ammonium chloride. The ether solution is dried with anhydrous sodium sulfate, and to the solution there are added 100 milliliters of ether, followed by 3.9 grams of cinnamaldehyde and 4 milliliters of 70% perchloric acid, and then, after the solution is cooled, it is saturated with dry hydrogen chloride gas. After standing in an ice-box, the solution is slowly diluted with 500 milliliters of ether and the precipitated crystals are collected and washed with ether thoroughly. The crystals are dissolved in dichloroethane and poured into ether to purify the same. The amount of purified crystals is 1.5 grams and they have a melting point of 158° to 161° C.

It has been discovered according to the invention that the compounds listed in Table 1 are sensitizing agents which can improve the photoconductivity and the spectrum characteristics of photoconductive polymers such as poly-N-vinylcarbazole, poly-3,6-dibromo-N-vinylcarbazole, brominated poly-N-vinylcarbazole, polyacenaphthylene and polyvinylanthracene. These polymers, except brominated poly-N-vinylcarbazole, are prepared in a per se well known method. The brominated poly-N-vinylcarbazole can be prepared by the following method: To the solution of 20 grams of poly-N-vinylcarbazole in 450 milliliters of chlorobenzene, there are added 18.44 grams of N-bromosuccinimide and 0.173 gram of benzoyl peroxide. The mixture is heated at 80° C. for 2 hours

while being stirred thoroughly and is poured into methanol to obtain a white polymer. The white polymer is dissolved in chlorobenzene and again poured into methanol for purification. The pure polymer thus obtained as a precipitate exhibits upon elementary analysis a halogen content of 29.87 weight percent which approximates the value calculated, i.e. 29.44 weight percent of the monobromosubstituted product from poly-N-vinylcarbazole. This indicates that the polymer obtained is a monobromo-substituted product. The degree of bromination varies from 50 mole percent to 200 mole percent according to reaction conditions.

The novel sensitizer comprising at least one compound from the group listed in Table 1 is dissolved in a suitable solvent, such as methanol, dichloroethane, methylene chloride, chloroform, or a combination thereof, and is added to the solution of the photoconductive polymer described above. The amount of the sensitizer added is from 0.01 to 3.0 weight parts in connection with 100 weight parts of the photoconductive polymer. Advantageously, the amount thereof is from 0.1 to 2.0 weight parts in connection with 100 weight parts of the photoconductive polymer.

The novel sensitizers according to the present invention differ from the well-known triphenylmethane dye-stuffs in the following two points:

First, the triphenylmethane dyestuffs have at least two radicals selected from the radical group comprising the amino, monomethylamino and dimethylamino radicals. The novel sensitizers according to the invention do not have such a radical.

Secondly, the novel sensitizers have an extreme ability to increase the photosensitivity of said organic photoconductors. For example, when the novel sensitizer, compound No. 2 (XIV), is used as a sensitizer of poly-N-vinylcarbazole, the photosensitive layer has a ten times higher sensitivity than the layer of poly-N-vinylcarbazole sensitized with a derivative (XV) of crystal violet which is a representative example of the triphenylmethane dyestuffs:



By suitable combinations of the novel sensitizers mentioned above, highly sensitive and panchromatic photosensitive layers are obtained easily.

For the preparation of the photoconductive insulating layer, a said solution of the photoconductive polymer and the carbonium salt in a suitable solvent is applied to the electroconductive support in per se usual manner, for example, by spraying by direct application, by means of blade coating, by means of whirler coating, etc., and then dried so as to produce a homogeneous photoconductive insulating layer on the electroconductive support. Operable solvents are benzene, toluene, chlorobenzene, dioxane, methylene chloride, dichloroethane and combinations thereof. Said solution may be incorporated with suitable plasticizers and/or organic colloids for improving the flexibility and strength of the photoconductive polymer. Operable plasticizers are as follows: chlorinated diphenyl, dimethyl phthalate, diethyl phthalate and octyl phthalate. Operable organic colloids are as follows: natural and synthetic resins, e.g. phenol resin, phenol resin modified

with rosin, polyvinyl acetal, polyvinyl butyral, polyvinyl cinnamate, polycarbonate resin. Operable materials for electroconductive supports may be made of any materials which satisfy the requirement of the electrophotographic art, e.g. metal plate or glass plate having NESO coating, plate or foils made of electrically conductive resins or coated with evaporated thin metal layer. If paper is to be used as a support for the photoconductive layer, pretreatment of the paper against penetration of the coating solution is advisable. The transparent support can produce a transparent electrophotographic plate, foil or film. After an electrostatic charge has been applied, i.e., after the layer has been charged positively or negatively by means of a corona discharge, the layer becomes light sensitive.

The reproduction of images by the electrophotographic method is carried out as follows: when the photoconductive layer has been charged by means of a corona discharge apparatus, the support with the sensitized layer is exposed to light under a master and is then dusted over in a per se known manner with a resin powder colored with carbon black. The image that now becomes visible can easily be wiped off. It can also be fixed by heating at about 120° C. From positive masters, positive images characterized by good contrast are produced.

It has been discovered according to the invention that more advantageous electrophotographic material can be prepared by a combination of brominated poly-N-vinylcarbazole and, as carbonium salt, at least one of the following compounds:

bis(4-methoxyphenyl)styrylcarbonium perchlorate,  
bis(4-methoxyphenyl)naphthyl(1')carbonium  
phenyl(4-methoxyphenyl)-4'-methoxynaphthyl(1')  
carbonium perchlorate,  
bis(4-methoxyphenyl)-2'-methoxynaphthyl(1')carbonium  
perchlorate,  
phenyl(4-methoxyphenyl)-2'-methoxynaphthyl(1')  
carbonium perchlorate,  
bis(4-methoxyphenyl)phenanthryl(9')carbonium  
perchlorate,  
phenyl(4-phenoxyphenyl)-4'-methoxynaphthyl(1')  
carbonium perchlorate,  
bis(4-methoxyphenyl)-4'-methoxystyrylcarbonium  
perchlorate,  
bis(4-methoxyphenyl)- $\omega$ -phenylbutadienylcarbonium  
perchlorate,  
bis(4-methoxyphenyl)- $\alpha$ -(4'-methoxyphenyl)-4''-  
methoxystyrylcarbonium perchlorate,  
phenyl-bis(4-methoxyphenyl)carbonium perchlorate,

and combinations thereof.

This invention is still further illustrated with reference to the following illustrative examples.

#### EXAMPLE 1

1 gram of polyacenaphthylene and 0.6 gram of, as a plasticizer, chlorinated diphenyl (commercially available as "Kanechlor"), are dissolved in 15 milliliters of dichloroethane. To the solution are added 0.5 milliliter of dichloroethane containing 0.005 gram of a carbonium salt corresponding to compound number 2, 3, 9, 11, 13, 14, 21 or 22 of Table 1. The solution is applied to an aluminum plate by means of whirler coating and is dried to form a layer of 3 $\mu$  in thickness. After said aluminum plate provided with the layer is charged negatively by means of corona discharge with a charging device maintained at approximately 6000 volts in the dark, it is placed under a positive master and is exposed to a 100 w. tungsten lamp at an illumination of 50 luxes, and the said plate is powdered over with a developer in a per se known manner. This developer consists of toner and carrier. The toner consists of a low melting point polystyrene, colophony and carbon black. The toner is mixed with a carrier

substance such that the toner becomes triboelectrically charged with a charge opposite to that produced on the plate. A positive image is produced and is fixed by slight heating. In Table 3, there are shown the optimum amounts of exposure in lux-second units.

TABLE 3

| Compound number: |               | Optimum exposure<br>(lux-sec.) |
|------------------|---------------|--------------------------------|
| 10               | No sensitizer | 200,000                        |
| 15               | 2             | 420                            |
| 15               | 3             | 84                             |
| 15               | 9             | 860                            |
| 20               | 11            | 92                             |
| 20               | 13            | 78                             |
| 20               | 14            | 84                             |
| 20               | 21            | 92                             |
| 20               | 22            | 81                             |

#### EXAMPLE 2

1 gram of poly-N-vinylcarbazole and 0.004 gram of a carbonium salt corresponding to compound number 2, 3, 6, 9, 11, 12, 13, 14, 16, 17, 19, 21, 22, 23, 24 or 25 of Table 1 are dissolved in 10 milliliters of dichloroethane.

The solution is applied to an aluminum plate and is dried to form a layer of 10 $\mu$  in thickness. An electrophotographic image is produced in the same way as that described in Example 1. In Table 4, there are shown the optimum amounts of exposure in lux-second units to produce exactly the original images.

TABLE 4

| Compound number: |               | Optimum exposure<br>(lux-sec.) |
|------------------|---------------|--------------------------------|
| 40               | No sensitizer | 20,000                         |
| 40               | 2             | 66                             |
| 40               | 3             | 32                             |
| 40               | 6             | 62                             |
| 40               | 9             | 74                             |
| 40               | 11            | 31                             |
| 45               | 12            | 62                             |
| 45               | 13            | 22                             |
| 45               | 14            | 32                             |
| 45               | 16            | 26                             |
| 45               | 17            | 52                             |
| 50               | 19            | 188                            |
| 50               | 21            | 24                             |
| 50               | 22            | 35                             |
| 50               | 23            | 22                             |
| 50               | 24            | 36                             |
| 55               | 25            | 24                             |

It is clear from Table 4 and FIGS. 5 to 7 that the novel sensitizers improve the photoconductivity and the characteristics of poly-N-vinylcarbazole.

#### EXAMPLE 3

1 gram of poly-3,6-dibromo-N-vinylcarbazole, 0.5 gram of chlorinated diphenyl (commercially available as "Kanechlor") and 0.004 gram of a carbonium salt corresponding to compound number 1, 2, 3, 4, 5, 6, 7, 8, 9, 10, 11, 12, 13, 14, 15, 16, 17, 18, 19, 20, 21, 22, 23, 24, 25, or 26 of Table 1 are dissolved in 10 milliliters of dichloroethane. This solution is applied to an aluminum plate by means of a blade coating and dried to form a layer of 14 $\mu$  in thickness. On these supports, electrophotographic images are produced in the same way as that described in Example 1. Table 5 shows the optimum amounts of exposure in lux-second units to reproduce exactly the original images.

11  
TABLE 5

| Compound number: | Optimum exposure<br>(lux-sec.) | 5   |
|------------------|--------------------------------|-----|
| No sensitizer    | 8000                           |     |
| 1                | 30                             |     |
| 2                | 58                             |     |
| 3                | 20                             |     |
| 4                | 42                             |     |
| 5                | 90                             |     |
| 6                | 56                             | 10  |
| 7                | 210                            |     |
| 8                | 92                             |     |
| 9                | 52                             |     |
| 10               | 64                             |     |
| 11               | 14                             | 15  |
| 12               | 48                             |     |
| 13               |                                | 14  |
| 14               |                                | 16  |
| 15               |                                | 180 |
| 16               |                                | 20  |
| 17               |                                | 42  |
| 18               |                                | 120 |
| 19               |                                | 132 |
| 20               |                                | 114 |
| 21               |                                | 16  |
| 22               |                                | 25  |
| 23               |                                | 18  |
| 24               |                                | 13  |
| 25               |                                | 17  |
| 26               |                                | 13  |
|                  | 40                             | 30  |

It is clear from Table 5 and FIGS. 8 to 10 that the novel sensitizers improve the photoconductivity and the spectrum characteristics of poly-3,6-dibromo-N-vinylcarbazole.

## EXAMPLE 4

1 gram of brominated poly-N-vinylcarbazole (mono-bromo-substituted product), 0.5 gram of polycarbonate resin (commercially available as "Panlite-C"), 0.3 gram of chlorinated diphenyl (commercially available as "Kanechlor") and 0.004 gram of a carbonium salt listed in Table 1 are dissolved in a mixed-solvent of 8 milliliters of chlorobenzene and 2 milliliters of dichloroethane. This solution is applied to an aluminum plate or to a cellulose diacetate film having a vacuum-evaporated film of cuprous iodide, by means of a blade coating and dried to form a layer of 12 $\mu$  in thickness. On these supports, electrophotographic images are produced in the same way as that described in Example 1. Table 6 shows the optimum amounts of exposure in lux-second units to reproduce exactly the original images.

TABLE 6

| Compound Number: | Optimum exposure on aluminum plate (lux-sec.) | Optimum exposure on CuI film (lux-sec.) |
|------------------|-----------------------------------------------|-----------------------------------------|
| No sensitizer    | 80,000                                        | 90,000                                  |
| 1                | 65                                            | 70                                      |
| 2                | 42                                            | 52                                      |
| 3                | 26                                            | 31                                      |
| 4                | 46                                            | 55                                      |
| 5                | 460                                           | 420                                     |
| 6                | 62                                            | 75                                      |
| 7                | 500                                           | 500                                     |
| 8                | 520                                           | 510                                     |
| 9                | 70                                            | 82                                      |
| 10               | 62                                            | 75                                      |
| 11               | 26                                            | 28                                      |
| 12               | 62                                            | 75                                      |
| 13               | 22                                            | 25                                      |
| 14               | 24                                            | 30                                      |
| 15               | 430                                           | 420                                     |
| 16               | 26                                            | 30                                      |
| 17               | 48                                            | 45                                      |
| 18               | 1,100                                         | 1,200                                   |
| 19               | 62                                            | 70                                      |
| 20               | 280                                           | 240                                     |
| 21               | 22                                            | 25                                      |
| 22               | 28                                            | 30                                      |
| 23               | 22                                            | 25                                      |
| 24               | 23                                            | 25                                      |

12

TABLE 6—Continued

| Optimum exposure on aluminum plate (lux-sec.) | Optimum exposure on CuI film (lux-sec.) |
|-----------------------------------------------|-----------------------------------------|
| 25                                            | 22                                      |
| 26                                            | 65                                      |
| 27                                            | 505                                     |
| 29                                            | 245                                     |
| 30                                            | 480                                     |
| 31                                            | 355                                     |
| 32                                            | 240                                     |
| 33                                            | 160                                     |
| 34                                            | 145                                     |
| 35                                            | 220                                     |
| 36                                            | 52                                      |
| 37                                            | 180                                     |
| 38                                            | 210                                     |
| 39                                            | 155                                     |
| 40                                            | 75                                      |
|                                               | 50                                      |
|                                               | 48                                      |
|                                               | 125                                     |
|                                               | 105                                     |

It is clear from Table 6 and FIGS. 1 to 4 that the novel sensitizers improve the photoconductivity and the spectrum characteristics of brominated poly-N-vinylcarbazole.

## EXAMPLE 5

1 gram of brominated poly-N-vinylcarbazole (mono-bromo-substituted product), 0.3 gram of polycarbonate resin (commercially available as "Panlite-C"), 0.3 gram of chlorinated diphenyl (commercially available as "Kanechlor"), 0.0024 gram of phenyl (4-methoxyphenyl)-4'-methoxynaphthyl(1')carbonium perchlorate (compound number 11), 0.0012 gram of bis(4-methoxyphenyl)-2'-methoxynaphthyl(1')carbonium perchlorate (compound number 13) and 0.0024 gram of phenyl (4-methoxyphenyl)2' - methoxynaphthyl(1')carbonium perchlorate (compound number 14), these three sensitizers are listed in Table 1, are dissolved in a mixed-solvent of 8 milliliters of chlorobenzene and 2 milliliters of dichloroethane. This solution is applied to an aluminum plate by means of a blade coating and dried to form a layer of 12 $\mu$  in thickness. Electrophotographic images are produced in the same way as that described in Example 1. The optimum exposure to the said plate is 20 lux-seconds and the said photosensitive layer has a panchromatic photosensitive layer in the region of visible spectrum as shown in FIG. 11.

Furthermore, the said solution is applied to glassine paper by means of a whirler coating and dried to form a layer of 3 $\mu$  in thickness. Electrophotographic images are produced in the same way as that described in Example 1. The optimum exposure to the said paper is 60 lux-seconds.

The invention has been described in detail with particular reference to preferred embodiments thereof, but it will be understood that variations and modifications can be effected within the spirit and scope of the invention as described hereinabove and as defined in the appended claims.

Having thus disclosed the invention, what is claimed is:

- An electrophotographic material comprising a conductive support layer and a photoconductive insulating layer, the latter comprising a combination of 100 weight parts of a photoconductive polymeric compound and 0.01 to 3.0 weight part of a sensitizer, said photoconductive polymeric compound comprising at least one compound selected from the group consisting of poly-N-vinylcarbazole, brominated poly-N-vinylcarbazole and polyacenaphthylene; said sensitizer comprising at least one compound selected from the group consisting of bis(4-methoxyphenyl)styrylcarbonium perchlorate, tris(4-methoxyphenyl)carbonium perchlorate, bis(4-methoxyphenyl)naphthyl(1')carbonium perchlorate, tris(4-methoxyphenyl)carbonium chloroferrate, phenyl-4-ethoxynaphthyl(1')carbonium perchlorate, phenyl(3,4-dimethoxyphenyl)biphenyl(4')carbonium perchlorate,

13

phenyl(4-methoxyphenyl)-4'-methoxynaphthyl(1') carbonium perchlorate,  
 phenyl-bis(4-ethoxyphenyl)carbonium perchlorate,  
 bis(4-methoxyphenyl)-2'-methoxynaphthyl(1')carbonium perchlorate,  
 phenyl(4-methoxyphenyl)-2'-methoxynaphthyl(1')carbonium perchlorate,  
 bis(4-methoxyphenyl)phenanthryl(9')carbonium perchlorate,  
 phenyl(3,4-diethoxyphenyl)phenanthryl(9')carbonium perchlorate,  
 phenyl(4-phenoxyphenyl)-4'-methoxynaphthyl(1')carbonium perchlorate,  
 bis(4-methoxyphenyl)-4'-methoxystyrylcarbonium perchlorate,  
 bis(4-methoxyphenyl)- $\omega$ -phenylbutadienylcarbonium perchlorate,  
 bis(4-methoxyphenyl)- $\alpha$ -(4'-methoxyphenyl)-4''-methoxystyrylcarbonium perchlorate,  
 bis(4-methoxyphenyl)- $\alpha$ -(4'-methoxyphenyl)- $\omega$ -phenylbutadienylcarbonium perchlorate,  
 phenyl-bis(4-methoxyphenyl)carbonium perchlorate,  
 bis(4-methoxyphenyl)-4'-phenoxyphenylcarbonium perchlorate,  
 tris(4-methoxyphenyl)carbonium chlorozincate,  
 tris(4-methoxyphenyl)carbonium fluoroborate  
 and combinations thereof.

2. An electrophotographic material according to claim 1, wherein said combination is a combination of 100 weight parts of brominated poly-N-vinylcarbazole and 0.1 to 2.0 weight parts of said sensitizer.

14

3. An electrophotographic material according to claim 1, wherein said combination is a combination of 100 weight parts of poly-3,6-dibromo-N-vinylcarbazole and 0.1 to 2.0 weight parts of said sensitizer.  
 5 4. An electrophotographic material according to claim 1, wherein said combination is a combination of 100 weight parts of poly-N-vinylcarbazole and 0.1 to 2.0 weight parts of said sensitizer.  
 5. An electrophotographic material according to claim 10 1 wherein said combination is a combination of 100 weight parts of polyacenaphthylene and 0.1 to 2.0 weight parts of said sensitizer.

## References Cited

## UNITED STATES PATENTS

|    |           |         |                        |        |
|----|-----------|---------|------------------------|--------|
| 15 | 3,037,861 | 6/1962  | Hoegl et al. -----     | 96—1.5 |
|    | 3,240,597 | 3/1966  | Fox -----              | 96—1.5 |
|    | 3,250,615 | 5/1966  | Van Allan et al. ----- | 96—1.7 |
|    | 3,274,000 | 9/1966  | Noe et al. -----       | 96—1.5 |
| 20 | 3,279,918 | 10/1966 | Cassiers et al. -----  | 96—1.5 |
|    | 3,418,116 | 12/1968 | Inami et al. -----     | 96—1.5 |
|    | 3,421,891 | 1/1969  | Inami et al. -----     | 96—1.6 |
|    | 3,464,819 | 9/1969  | Inami et al. -----     | 96—1.5 |

## OTHER REFERENCES

- 25 Nelson, "An Effect of the Anion on the Conductive Properties of Triphenyl Methane Dye Salts," J. Chem. Physics, vol. 20, pp. 1327, 1328, August 1952.

30 CHARLES E. VAN HORN, Primary Examiner

U.S. Cl. X.R.

96—1.5